

Dec. 17, 1940.

R. C. BENNER ET AL

2,225,193

ABRASIVE WHEEL

Filed Sept. 15, 1937

3 Sheets-Sheet 1



BY

INVENTOR  
RAYMOND C. BENNER  
WILLIAM G. SOLEY

*R. C. Benner*

ATTORNEY.

Dec. 17, 1940.

R. C. BENNER ET AL

2,225,193

ABRASIVE WHEEL

Filed Sept. 15, 1937

3 Sheets-Sheet 2



BY

INVENTOR.  
RAYMOND C. BENNER  
WILLIAM G. SOLEY

*Raymond C. Benner*  
ATTORNEY.

Dec. 17, 1940.

R. C. BENNER ET AL

2,225,193

ABRASIVE WHEEL

Filed Sept. 15, 1937

3 Sheets-Sheet 3



BY

INVENTOR.  
RAYMOND C. BENNER  
WILLIAM G. SOLEY

*R.C.Benner*

ATTORNEY.

## UNITED STATES PATENT OFFICE

2,225,193

## ABRASIVE WHEEL

Raymond C. Benner and William G. Soley,  
 Niagara Falls, N. Y., assignors to The Carbo-  
 rundum Company, Niagara Falls, N. Y., a cor-  
 poration of Delaware

Application September 15, 1937, Serial No. 164,028

8 Claims. (Cl. 51—206)

This invention relates to improved abrasive articles, and particularly to abrasive articles in which diamonds or other costly materials constitute at least in part the abrasive element. 5 This invention pertains especially to articles in which the active abrasive element is bonded to form aggregates or inserts which are distributed in a matrix material to form abrasive products of improved cutting characteristics. 10 Heretofore, in the making of grinding wheels in which diamonds are used as the abrasive, the bonding of the diamonds has been mostly confined to such plastic materials as synthetic resins and sintered metals which can be consolidated 15 into a dense and practically non-porous mass. Difficulty has been experienced in the usual ceramic bonding of diamond abrasive wheels in that there is a break-down of the bond during cutting. This sort of break-down is very desirable with cheap abrasives, such for example, as silicon carbide or fused alumina, etc., but such a break-down of the bond when diamonds are used as the abrasive is not desirable. This is due to the fact that in order to be practical in 20 operation and to secure sufficient service to warrant the cost, the diamonds must be retained in the cutting surface of the wheel over a long period of time.

The present invention relates to the making of 30 abrasive grinding wheels or discs using diamonds, or other of the more costly grinding media wherein the abrasive particles are incorporated in bonded aggregates or inserts. These inserts or aggregates are then positioned or distributed in 35 and bonded with a matrix of supporting material to form the working surface or edge of the final grinding wheel or disc. The material used for bonding these inserts may be any type of bond such as ceramic, metallic, rubber, or resinous in character. The supporting matrix material is usually, although not necessarily so, a bond of different characteristics than the bond for the insert, and depends upon the type of wheel being made and the use to which it is to be 40 put. This use of a matrix material different in characteristics from the bond used in the insert gives the resulting wheel cutting properties which are distinct from standard wheels of uniform surface and constitute an improvement in cutting rates and efficiency ratios over such wheels. The properties of different wheels can be altered to adapt the wheel to various applications by interchange of different insert-bonds with different types of matrices in a way impossible with 50 wheels of a solid uniform grinding face. This 55

matrix material may be any one of a number of substances, including rubber, ceramic, resinous or metallic compositions, etc.

One of the principal objects of the present invention is to provide ways for the more economic 5 use of diamonds in the making of grinding wheels having improved cutting rates and efficiencies. It is the purpose to attain these improved properties while actually using less diamonds than have hitherto been used for making wheels of 10 similar size.

Another object of the present invention is the proposed use of diamonds in larger wheels than have heretofore been made with diamonds, such 15 wheels to possess diamond-grinding surfaces greater and more extensive than have been previously considered feasible.

A further object is the provision of diamond 20 wheels of increased thickness presenting wide peripheral grinding surfaces without excessive use of diamonds. One of the proposed methods of accomplishing this is by use of thin overlapping annular segments embedded in the wheel periphery.

Another object is the production of diamond 25 grinding wheels capable of a vast range of cutting characteristics each adaptable to a specific type of work, this to be accomplished by careful selection of insert-bond and matrix and proper use of one with the other. 30

Other objects and advantages of the invention will become apparent during the course of the following description.

The nature of the present invention is better 35 illustrated by the following drawings in which embodiments of the invention are shown:

Figure 1 is a plan view of a disc wheel showing the bonded inserts or discs arranged in the cutting surface of the wheel.

Figure 2 is a cross section on the line II—II 40 of Figure 1.

Figure 3 is a plan view of a cut-off wheel using alternately spaced diamond bonded inserts in both sides of the wheel.

Figure 4 is a cross section along the line IV—IV 45 of Figure 3.

Figures 5 and 6 are plan views of further modifications of wheels containing bonded abrasive inserts.

Figures 7 and 8 are cross sections along the 50 lines VII—VII and VIII—VIII of Figures 5 and 6, respectively.

Figure 9 is a plan view of a cut-off wheel showing a modification of the positioning of the inserts.

Figure 10 is a plan view of another modification in the shape of inserts used.

Figure 11 is a cross section along the lines XI—XI of Figure 10.

5 Figure 12 is a side plan view of a grinding wheel showing the use of diamond bonded overlapping annular segments embedded about the peripheral grinding surface.

10 Figure 13 is a front plan view of the wheel shown in Figure 12.

Figure 14 is a plan view of a large size diamond wheel using overlapping inserts to present a large broad side grinding surface.

15 In all of the drawings like numerals refer to the same thing throughout the figures. Numeral 1 is the bonded insert or aggregate which contains the diamond abrasive particles, and 2 is the matrix material or secondary bond in which the abrasive inserts 1 are embedded. 3 is the 20 backing or support used in some types of wheels to which the shaped matrix 2 is cemented or fastened and serves as a means for fastening to the grinding apparatus by means of bolts through holes 4.

25 Figure 1 and 2 the inserts 1 are shown as ceramic bonded diamond particles while the matrix 2 is a metallic material. The backing is made up of a resinous material such as Bakelite or other thermo-setting resin.

30 Figures 3 and 4 show a modification of a cut-off wheel using inserts according to the present invention. The inserts 1 in this example are metal-bonded diamond particles and the remainder of the wheel body is made up of a resin bonded cheap abrasive such as fused alumina or silicon carbide grain.

35 Figures 5 and 7 illustrate a thin grinding wheel with inserts 1 of such shape and position that the matrix material 2 may be dressed down between the diamond-containing inserts 2 after periods of use without any great inconvenience. The inserts are shown here of resin bonded diamonds, and the matrix of rubber bonded abrasive such as silicon carbide or fused alumina.

40 Figures 6 and 8 illustrate a modification of the type of wheel shown in Figures 1 and 2, using a different shaped insert 1, and like the wheel in Figures 5 and 7 may be easily dressed down. In this modification the inserts are shown of a metal bonded abrasive with the matrix material 2 also composed of a metallic composition.

45 Figure 9 is a plan view showing a still further modification of a wheel in which the inserts 1 are positioned in more or less spiral form.

50 Figures 10 and 11 illustrate a wheel having wedge shaped metal bonded inserts 1 positioned in the face of a rubber matrix 2.

55 Figures 12 and 13 are side and front plan views respectively of a grinding wheel in which the periphery or edge of the wheel constitutes the grinding surface and whose edge is of considerable thickness in order to present a broad working surface. The diamond-containing inserts 1 are in the form of thin annular segments having an outside curvature corresponding to the outside circumference of the completed wheel and are embedded in the matrix material 2 to form part of the working surface of the wheel. As can be seen in the front plan view these inserts or segments are staggered and overlap laterally. In the illustrations shown the inserts are ceramic-bonded and the matrix is of a resinous composition.

60 One method by which we make these annular segments for use in wheels as shown in Figures

12 and 13 is to mold and press complete thin rings of the composition of the inserts and having the same outer circumference as that of the final grinding wheel desired and slightly over half the thickness of the wheel in which they are to be incorporated. After final firing or curing these complete annular rings are broken or cut into segments of the length desired for embedding in the surface of the wheel.

65 In Figure 14, the inserts 1 of ceramic bonded diamonds are overlapping and embedded in the rubber matrix 2 to form a large broad top dressing surface of considerable area.

70 According to one method of making up wheels containing bonded diamond inserts, the inserts 15 are pressed to shape and cured or fired before incorporation in the wheel. However, these inserts, if of approximately the same maturing temperature as the matrix material, may be made up at the same time the matrix material 20 is mixed and simultaneously pressed and fired with it by the use of dividing partitions in the mold, without departing from the scope of this invention. For example, if a wheel similar to that illustrated in Figures 6 and 8 is to be made up and the materials of the matrix and abrasive inserts have approximately the same maturing temperatures then both mixes may be made in separate batches at the same time and in setting up the mold, partitions may be temporarily 25 placed in the mold and the two different mixes 30 placed in their respective positions, the partitions carefully withdrawn and the whole wheel 35 pressed in a single operation and later fired.

40 Where the inserts are formed prior to incorporation in the matrix of the wheel the following method may be used to properly position the inserts in the finished wheel, although this is not the only method which may be used within the scope of my broad invention. A piece of 45 paper or other material carrying the desired design is placed on the bottom of the mold. This paper has on it a design showing the desired location of the inserts which are then positioned accurately according to the design on this base 50 paper. The inserts may be held in position in contact with the paper by the presence on the paper of a small amount of transparent adhesive such as glue or resin just sufficient to hold the insert firmly while the loose matrix material 55 is poured into the mold and leveled off, after which the wheel is pressed and fired or cured. This method is especially desirable where inserts are intricately positioned, such as for example those shown in Figure 9. Careful positioning of 60 the inserts not only improves the appearance of the wheel but keeps it in better balance and helps to insure utilization of the abrasive in the desired manner. Where positioning on opposite sides of the wheel is desired, as in Figures 3 and 4, 65 it is most readily accomplished on the second side by use of a perforated template.

70 As a specific example of making ceramic bonded diamond inserts abrasive particles are mixed with the bond in the following proportions 65 and pressed at approximately 8000 lbs./sq. in. and after drying are fired at 1300° C.

| 1.                   | Per cent | 70 |
|----------------------|----------|----|
| 80-140 grit diamonds | 40       |    |
| 400 grit alumina     | 40       |    |
| Bond                 | 20       |    |

75 These inserts are held together by a temporary binder which is burned out by firing up to 500° C. 75

in an oxidizing atmosphere, after which they are fired under reducing conditions to 1300° C.

2.

Per cent

|                           |    |
|---------------------------|----|
| 5 Diamonds 80-140 grit    | 40 |
| 50% 100 and finer alumina | 40 |
| 50% 400 grit alumina      |    |
| Bond                      | 20 |

10 The ceramic bond used in the above two mixes is exemplified by the following two bonds, although many other ceramic compositions may be used which would work satisfactorily.

1.

|                 |        |
|-----------------|--------|
| 15 17.4% Kaolin |        |
| Soda ash        | 1.06%  |
| Potash          | 1.51%  |
| Flint           | 54.66% |
| 82.6% Borax     | 32.23% |
| Whiting         | 4.63%  |
| MgO             | 2.38%  |
| ZnO             | 3.53%  |

or

2. A glass of the following composition:

|                                |      |
|--------------------------------|------|
| 25 SiO <sub>2</sub>            | 74.2 |
| B <sub>2</sub> O <sub>3</sub>  | 11.4 |
| Na <sub>2</sub> O              | 12.0 |
| K <sub>2</sub> O               | .1   |
| 30 CaO                         | .3   |
| Al <sub>2</sub> O <sub>3</sub> | 2.0  |

The following mix is an example of one which has been found very satisfactory in making metal bonded diamond inserts.

35 1.

|                           |    |
|---------------------------|----|
| Per cent                  |    |
| Bond (20% tin—80% copper) | 80 |
| 80-140 grit diamonds      | 10 |
| 180 grit silicon carbide  | 10 |

40 After thorough mixing of the ingredients the mix is screened through a 60 mesh screen to prevent balling up of the metal bond and then pressed at 10,000-100,000 lbs./sq. in., after which they are 45 burned at 700-750° C. under an atmosphere of illuminating gas. During firing the inserts or pellets are placed between bats and weighted down with a weight of a few pounds on the upper bat to prevent warping. After cooling they are 50 removed and cleaned off with a wire brush and washed with a 5% solution of sodium cyanide.

After the diamond inserts have been made and properly burned or matured, they are positioned in a ring mold and the matrix or supporting 55 mix filled in around the inserts, leveled off, and pressed at 10,000-75,000 lbs./sq. in. The wheel is then removed from the ring mold and burned in a furnace between bats to prevent warping. The following two mixes are given as highly 60 satisfactory examples of metal bonds which may be used as the matrix material and are fired using the same temperature and atmosphere as the metallic inserts given above.

1.

Per cent

|        |    |
|--------|----|
| Copper | 88 |
| Tin    | 12 |

2.

Per cent

|        |    |
|--------|----|
| Copper | 92 |
| Tin    | 8  |

70 Instead of using ceramic compositions or metallic bonds for either the inserts or matrix of the 75 wheel as shown above, either the matrix or in-

serts may be made up using a rubber bond. Although smoked sheet rubber is given below in the specific example, a mix may be made up using either dispersed or decomposed rubber with good results.

For making rubber bonded diamond abrasive inserts the following mix is given as a specific example:

|                                                                                          |      |
|------------------------------------------------------------------------------------------|------|
| Per cent                                                                                 |      |
| 100 parts smoked sheet rubber, 50 parts sulphur, 1 part accelerator, 0.5 part zinc oxide | 10   |
| 80-140 grit diamonds                                                                     | 42.5 |
| 400 grit alumina                                                                         | 42.5 |

15 Inserts of the above ingredients are pressed and partially cured for 5 minutes at 120 lbs. steam pressure after which they may be removed, placed in a ring mold, rubber matrix material as specified below added, and the inserts and matrix combined given a further press cure for 55 minutes at 120 lbs. steam pressure. Instead of curing in the press the matrix and insert after short pressing may be oven cured 4 hours at 300° F. It should be understood that rubber bonded inserts may be used with other matrix material 25 such as resins, in which event the inserts may be completely cured before incorporation in the matrix.

The following composition is a typical mix for use as a rubber matrix material:

|                     |     |
|---------------------|-----|
| Parts               |     |
| Smoked sheet rubber | 100 |
| Sulphur             | 50  |
| Accelerator         | 1   |
| Zinc oxide          | 0.5 |
|                     | 35  |

40 In making inserts of a resin bonded abrasive I have found that phenol-formaldehyde resins are highly satisfactory. As an example of a resinous insert composition the following has worked out well:

|                                  |    |
|----------------------------------|----|
| Per cent                         |    |
| Powdered reactive phenolic resin | 20 |
| 80-140 grit diamonds             | 40 |
| 400 grit alumina                 | 20 |
| 100 and finer alumina            | 20 |
|                                  | 45 |

45 In making inserts of the above mix the abrasive is first mixed thoroughly and moistened with furfural, after which the powdered resin is added to give a free-flowing mix. This mix is cold 50 pressed and the inserts as made are baked in an oven by bringing them slowly up to 350° F. over a period of 24 hours and holding at that temperature for 2 hours and then cooling.

The following is a specific example of a resin 55 mix which has been found adaptable for a matrix material for bonding abrasive inserts. In forming the matrix shapes of such a resinous compound the inserts are placed in the mold, the powdered mix filled about the inserts, hot pressed 60 30 minutes at 140 lbs. steam pressure, cooled under pressure, removed from the mold and baked in an oven by taking them slowly up to 350° F. over a period of 24 hours and holding at that temperature for 2 hours.

|                                   |          |
|-----------------------------------|----------|
| 65                                | Per cent |
| Phenol-formaldehyde molding power | 20       |
| Flint filler                      | 80       |

70 In the specific embodiments of wheels herein illustrated reference was made to the desirability 70 in certain cases of dressing down the wheel after periods of use. This is especially applicable to wheels in which the diamonds are embedded in inserts or aggregates in which the bond of the insert is of a porous, brittle type to produce a 75

free, rapid cutting action. This bond, if used alone wears away so rapidly as to cause an undesirable high wheel loss, but when used together with a matrix of tougher material this 5 wheel loss is reduced by protection of the more fragile insert-bond by the tougher matrix composition. To explain more fully, when the wheel is first put in use the surface of the insert is approximately flush with the surface of the 10 matrix, but the bond of the insert quickly wears away to a slight extent exposing a number of diamond cutting surfaces which protrude above the bond. However, the tougher matrix material does not wear away as rapidly and supports 15 the work sufficiently to prevent further immediate wearing away of the insert-bond and ripping out of the diamond particles, although undergoing wear sufficiently to permit the partly exposed diamond particles to cut freely. At the 20 same time this slightly lowered bond surface of the insert allows for a chip clearance not otherwise present and an opportunity for the detritus to be easily carried away. After the abrasive insert has worn down so far as to materially 25 diminish or retard the cutting action it becomes desirable to cut or dress down the matrix slightly. For this purpose it is advantageous to be able to apply a dressing tool which can cut back the matrix without also striking the abrasive 30 insert. This is most readily accomplished where the configuration of the inserts is as shown in Figure 6 for example where the dressing is done in two steps, first the central portion and then the "spokes" between the inserts. 35 By the use of bonded inserts in making diamond grinding wheels many advantages are obtained. For example, in the pressing of diamond wheels it is quite essential for the best results that the wheels be pressed at relatively high pressures, and when the whole wheel is made up 40 as hitherto carried out, large massive presses and expensive pressing equipment is necessary to form the wheel. By the proposed method of using inserts of comparatively small area individually with respect to the entire wheel area, 45 these high pressures can be reached with the far less costly pressing apparatus. In the case of small buttons or pellet-shaped inserts, pressures in the neighborhood of several thousand 50 pounds per square inch may be had by ordinary hand pressure apparatus. This ability to obtain highly compressed bonded diamond segments or inserts without elaborate pressing equipment constitutes a marked economic saving. 55 A further saving is realized by the fact that instead of diamonds being used throughout the entire wheel, only a portion of the wheel abrading surface contains diamonds. Not only are less diamonds used, but this accomplished while 60 at the same time wheels are made having a free cutting action without an extravagant wheel loss. 65 Grinding wheels or disks made up according to the present invention having diamond particles present only in inserts placed in the abrading surface of the wheel instead of being incorporated in the entire grinding surface not only do not suffer any loss in cutting rate or efficiency in comparison with a wheel having diamonds in the entire working face, but in fact, show a definite 70 increase in the cutting rate and an improvement in the efficiency over such diamond cutting wheels. Wheels using considerably less of diamond particles but made up with spaced inserts or aggregates show a higher efficiency and cutting rate than similar bonded wheels using a

greater amount of diamonds spread throughout the cutting surface. This is accomplished without any detrimental effect upon cutting characteristics.

By the use of a free-cutting bond for the inserts which is backed up or supported by a tougher matrix material the cutting properties such as cutting rate and efficiency ratio of the wheel is improved by the use of inserts in place of the standard uniform grinding surface as commonly used regardless of the purpose or application to which the wheel is put. By efficiency ratio we mean the resulting figure obtained by dividing the grams of material being ground which is removed per minute by the grams of wheel loss 15 per minute. A preferred wheel is one which shows a high efficiency ratio. Wheels made with inserts have exhibited extremely high efficiency ratios as well as greatly improved cutting rates over standard wheels regardless of the work or 20 purpose of the wheel.

Some explanation has been suggested above as to the reason for this improved cutting action and efficiency. It has, generally speaking, been found advantageous to use an insert bond which 25 possesses the property of breaking away freely around each diamond particle and exhibiting some signs of brittleness, although having sufficient tenacity to keep the diamond particles from ripping out. The most desirable bond to be used 30 varies, dependent upon the material being ground and other factors just as in the case of ordinary grinding wheels. On the other hand, the bond for the matrix or remainder of the surface of the wheel is chosen usually so that it possesses 35 greater toughness and strength than the insert bond, has an improved abrading or wear resistance, and acts as a support to prevent undue break-down of the more fragile insert material. In general rubber matrices are indicated 40 where some degree of resilience is desired, resin matrices where a stiff somewhat brittle action is desired, and metal matrices for use on hard materials such as ceramic products under certain 45 circumstances.

In the use of diamonds as a grinding medium in wheels it has been found extremely difficult to find a bond which satisfactorily wet the diamond surfaces so as to tenaciously hold the diamonds in place and give a desirable cutting action and also possessed the toughness and resilience necessary to be used to make up the entire body of a wheel of any considerable size. This, in addition to the excessive cost entailed in using diamonds promiscuously throughout the wheel, 55 has limited the use of diamonds to wheels of smaller size. By the proposed use of inserts, a wheel body may be used which possesses properties suitable for forming larger wheels without regard to its ability to tightly bond diamonds and 60 a different bond especially adapted for bonding diamonds than used for the inserts. This use of a matrix or body different in properties from the insert bond thus aids in the production of wheels of increased cutting rate and efficiency 65 in addition to the economic reason of saving on the amount of diamonds necessary. Then too by the correct choice and combination of insert bond and matrix bond any desirable cutting action may be obtained over a substantial range of differentiations.

While several specific examples and mixes have been herein given to show the actual working of this invention, we do not wish to be limited to these embodiments solely as illustrated. We 75

wish to point out that by judicious selection of the proper bond for the insert and a like careful selection of matrix bond that a large range of cutting actions can be had, depending on the proposed application of the wheel. In other words, 5 ceramic, resinous, metallic, or rubber bonds may be interchangeably used in the insert or matrix at will, depending on the type of wheel desired. Also, although we have referred for the most part 10 to the use of diamonds as the abrasive element, we wish it understood that other costly abrasives such as boron carbide and the like may be used without departing from the spirit of the present invention.

15 We claim:

1. As an article of manufacture, an abrasive article comprising ceramic-bonded diamond containing inserts embedded in a rigid, non-abrasive supporting matrix the surface of which is substantially flush with the grinding surface of the adjoining inserts.

2. As an article of manufacture, an abrasive article comprising ceramic-bonded diamond containing inserts embedded in a metallic matrix.

25 3. As an article of manufacture, an abrasive article comprising ceramic-bonded diamond aggregates bonded together in a metallic matrix.

4. As an article of manufacture, an abrasive 30 wheel comprising ceramic-bonded diamond-containing inserts circumferentially spaced about the periphery of the wheel and embedded in a rigid, non-abrasive supporting matrix forming the body

of said wheel said matrix having greater wear-resistance than bond of said inserts.

5. As an article of manufacture, an abrasive wheel comprising ceramic-bonded diamond-containing inserts circumferentially spaced about 5 the periphery of the wheel and embedded in a rigid, non-abrasive supporting matrix forming the body portions of said wheel said matrix having greater wear-resistance than bond of said inserts, and said inserts being so shaped and 10 positioned as to permit dressing of the body of the wheel after periods of use.

6. As an article of manufacture, an abrasive article comprising ceramic-bonded diamond-containing inserts, embedded in a rigid, non-abrasive, 15 body portion, said body portion having greater wear-resistance than the bond of said inserts.

7. As an article of manufacture an abrasive article comprising diamond-containing inserts bonded within by a bond having the free-cutting, 20 friable characteristics of a ceramic bond, said inserts being embedded in a rigid supporting matrix of non-abrasive material, the surface of which is substantially flush with the grinding surface of the adjoining inserts.

25 8. As an article of manufacture an abrasive article comprising ceramic-bonded diamond-containing inserts imbedded in a rigid non-abrasive organic supporting matrix, the surface of which is substantially flush with the grinding surface 30 of the adjoining inserts.

RAYMOND C. BENNER.  
WILLIAM G. SOLEY.